

## UNITED STATES PATENT OFFICE

2,180,520

PROCESS FOR THE SEPARATION OF NICKEL  
FROM COPPER

Guenther Hamprecht and Gustav Pauckner, Ludwigshafen-on-the-Rhine, Germany, assignors to I. G. Farbenindustrie Aktiengesellschaft, Frankfort-on-the-Main, Germany

No Drawing. Application April 1, 1939, Serial No. 265,604. In Germany April 7, 1938

2 Claims. (Cl. 75—119)

The present invention relates to a new process for the separation of nickel from copper.

For the recovery of nickel from ores which contain copper in addition to nickel it has already been proposed first to melt a so-called nickel-copper matte and then to treat this with copper chloride solution which may be prepared by leading chlorine into a cuprous chloride solution. The nickel chloride-cuprous chloride solution thus obtained is then worked up electrolytically into nickel and copper, copper chloride thus being simultaneously recovered which serves for the treatment of further amounts of nickel-copper matte. This process has, however, not hitherto found use industrially because the electrolysis of the cuprous chloride-nickel chloride solution is attended by difficulties and the copper obtained by the electrolysis of the chloride solution is not pure enough for many purposes.

We have now found that the said difficulties can be avoided and a complete separation of nickel from copper can be obtained in a simple manner by dividing the nickel chloride-cuprous chloride solution obtained by treating the nickel-copper matte with cupric chloride solution and reforming in one part of the said nickel chloride-cuprous chloride solution by treatment with chlorine, the cupric chloride necessary for the treatment of further amounts of nickel-copper matte, and precipitating from the other part of the solution the copper by the action of nickel-copper matte.

It is preferable to use a matte the sulphur content of which amounts at the most to one third of the copper content. The precipitated high-percentage copper mass may be worked up to pure copper. During the action of the solution containing cuprous chloride on the nickel-copper matte (cementation), the amount of nickel equivalent to the copper passes into solution and there is obtained a nickel chloride solution practically free from copper which may be worked up electrically to nickel and chlorine without difficulty. The cementation is preferably carried out at elevated temperatures, for example at from 90° to 100° C. or higher, if desired under pressure.

The chlorine formed by the electrolysis is led into the part of the solution separated for the working up of the fresh matte and thus re-forms the amount of cupric chloride necessary for the dissolving process.

By the said new method of working it has been rendered possible to separate the copper from nickel in a cyclic process which proceeds quite

smoothly whichever the composition of the matte to be worked up may be. According to the equations:



the quantities of copper which is carried in a cycle in the form of copper chloride, are 2.17 metric tons for every metric ton of nickel to be produced and 1 metric ton for every metric ton of copper to be produced, i. e. 3.17 metric tons of copper in all. This quantity of copper, as cuprous chloride, is capable of binding 1.8 metric tons of chlorine. After such combination with chlorine, the solution resulting in the cyclic process contains 3.17 metric tons of copper in the form of cupric chloride. By the aid of the solution thus obtained the nickel and copper content

3.17

$2.17x + y$

metric tons of matte, containing  $x$  per cent of nickel and  $y$  per cent of copper may then be completely dissolved out. The resulting solution which contains nickel chloride and cuprous chloride is divided in such a proportion, that the part to be carried in a cycle again contains 3.17 metric tons of copper per each ton of nickel and copper to be dissolved out from the matte, whereas the other part of the solution which is to be carried to further treatment for precipitation of the copper contains an amount of nickel and copper which corresponds to that contained in the lixiviated matte. This part is then treated with nickel-copper matte, containing  $x_1$  per cent of nickel,  $y_1$  per cent of copper and  $z$  per cent of sulphur,  $z$  corresponding preferably to at the most  $\frac{1}{3}y_1$ . According to the equation:



for 1 part of copper in the solution

$\frac{46}{x_1}$  parts of the latter matte

are to be applied.

From the solution of nickel chloride thus obtained, on electrolysis 1.8 metric tons of chlorine, i. e. the amount required for the cyclic operation, is re-formed.

The following examples will further illustrate the nature of this invention but the invention is not restricted to these examples.

## Example 1

10.4 metric tons of nickel-copper matte containing 50 per cent of nickel, 27 per cent of cop-

per and 22 per cent of sulphur are treated with a solution containing 14.1 metric tons of copper as cupric chloride and 26.1 metric tons of nickel as nickel chloride. From the nickel-copper matte 5 there thus pass into solution 5.2 metric tons of nickel and 2.8 metric tons of copper, while the sulphur remains undissolved. Should all the copper and nickel not yet be dissolved out from the matte, the residue is preferably subjected again 10 to a short treatment with fresh solution. The resulting solution then contains the whole of the copper (16.9 metric tons) as cuprous chloride and 31.3 metric tons of nickel as nickel chloride. The solution is divided into two parts so that one part 15 again contains 14.1 metric tons of copper and after treatment with chlorine for the purpose of converting the cuprous chloride to cupric chloride is again capable of lixiviating 10.4 tons of nickel-copper matte. The other part, which corresponds 20 to the freshly-introduced nickel and copper, is diluted with water and then treated with 3 metric tons of a nickel-copper matte containing 43 per cent of nickel, 47 per cent of copper and 8 per cent of sulphur. The 1.3 metric tons of nickel 25 contained in the matte thus passes down to a few per cent into solution, while the 2.8 metric tons of copper contained in the solution are precipitated to a great extent.

The resulting nickel chloride solution is freed 30 in known manner from the remainder of the copper and traces of sulphur and then electrolysed. The nickel is thus deposited and at the same time chlorine is set free in an amount of 7.9 metric tons. This chlorine is then brought 35 into action with the part of the solution containing 14.1 metric tons of copper as cuprous chloride, the latter thus being converted to cupric chloride.

*Example 2*

40 7.86 metric tons of a nickel-copper matte containing 42 per cent of nickel and 47 per cent of copper is lixiviated with a chloride solution containing 10.84 metric tons of copper and 9.63 metric tons of nickel. 3.3 metric tons of nickel 45 and 3.69 metric tons of copper thus pass into solution. A part of the resulting solution, which is measured to correspond to a content of 10.84 metric tons of copper, is treated with chlorine to convert the cuprous chloride again into cupric chloride and is then used for the working up of 50 a further 7.86 metric tons of nickel-copper matte. The other part is treated with a nickel-copper matte which has already been used for the precipitation of copper from a solution but which 55 still contains nickel. This residual amount of nickel is by this treatment practically completely dissolved out, while the solution is only partly decoppered. After separating the residue, the solution is treated with 4.05 metric tons of fresh 60 matte of the composition above specified, so that now the nickel is present in the matte in excess as compared with the copper in the solution. By this after-treatment, the solution is completely freed from copper. The residue, which still contains nickel, is then used again for the partial 65 removal of copper from fresh solution. The resulting nickel chloride solution is practically completely free from copper.

*Example 3*

70 30 cubic meters of an aqueous solution, at a temperature of 60° C. which contains per liter 100 grams of common salt, 292 grams of cupric

chloride and 386 grams of nickel chloride is brought together in a stirring vessel with 3 metric tons of finely broken or ground nickel-copper matte containing 42 per cent of nickel, 47 per cent of copper, 0.6 per cent of iron and 10 per cent of sulphur. The solution heats up spontaneously and very rapidly to 100° C. After a short time it may be filtered off from the residue which consists mainly of pure sulphur. The presence of common salt in the solution serves to prevent 10 the precipitation of cuprous chloride.

The solution has 10 cubic meters of water added to it and is then divided. 30 cubic meters of the solution are chlorinated and, after the addition of 750 kilograms of common salt and 367 kilograms of nickel as chloride, again caused to act 15 on 3 metric tons of fresh nickel-copper matte.

The remainder, 10 cubic meters, is heated by the leading in of steam to from 90° to 100° C. and treated with 1800 kilograms of nickel-copper 20 matte of the above composition, whereby the copper is precipitated within 4 hours.

Any remainders of copper still present in the solution are precipitated with barium sulphide. At the same time any sulphate present in solution 25 is precipitated. Iron which has not yet been separated may be removed by the action of alkalies, such as soda, or nickel hydroxide. The resulting pure nickel chloride solution is further worked up by electrolysis. The chlorine thus set 30 free may serve for chlorinating the cuprous chloride solution.

What we claim is:

1. In a process for the separation of nickel from copper contained in nickel-copper matte 35 by treating the said matte with copper chloride solution with the formation of nickel chloride and cuprous chloride and converting the cuprous chloride with chlorine into cupric chloride and employing the solution thus obtained for the treatment of further amounts of nickel-copper matte, the steps which comprise dividing the nickel chloride-cuprous chloride solution obtained by treating the nickel-copper matte with cupric chloride solution, and re-forming in one part of the said nickel chloride-cuprous chloride solution 40 by treatment with chlorine the cupric chloride necessary for the treatment of further amounts of nickel-copper matte, and precipitating from the other part of the solution the copper by the action of nickel-copper matte. 50

2. In a process for the separation of nickel from copper contained in nickel-copper matte by treating the said matte with copper chloride solution with the formation of nickel chloride and cuprous chloride and converting the cuprous chloride with chlorine into cupric chloride and employing the solution thus obtained for the treatment of further amounts of nickel-copper matte, the steps which comprise dividing the nickel chloride-cuprous chloride solution obtained by treating the nickel-copper matte with cupric chloride solution, and re-forming in one part of the said nickel chloride-cuprous chloride solution 55 by treatment with chlorine the cupric chloride necessary for the treatment of further amounts of nickel-copper matte, and precipitating from the other part of the solution the copper by the action of a nickel-copper matte, the sulphur content of which amounts at the most to one third 60 of the copper content. 65

GUENTHER HAMPRECHT,  
GUSTAV PAUCKNER.